

# UNITED STATES PATENT OFFICE.

HUBERT HERKOMER AND HENRY THOMAS COX, OF BUSHEY, ENGLAND.

## MODE OF PREPARING ARTISTIC PRINTING-SURFACES.

SPECIFICATION forming part of Letters Patent No. 556,975, dated March 24, 1896.

Application filed April 3, 1895. Serial No. 544,259. (No specimens.) Patented in England November 23, 1891, No. 20,346.

*To all whom it may concern:*

Be it known that we, HUBERT HERKOMER, R. A., and HENRY THOMAS COX, of Bushey, in the county of Herts, England, have invented 5 certain new and useful Improvements in the Mode of Preparing Artistic Printing-Surfaces, of which the following is a specification, and for which we have obtained Letters Patent of Great Britain, No. 20,346, dated November 10 23, 1891.

The object of the present invention is to prepare, by the aid of the electrotype process, printing-surfaces (in a simple and expeditious manner) which will reproduce, by printing, the artistic touches obtainable only from 15 the hand of the artist.

In carrying out our invention we provide a smooth ground—for example, a copper-plate, such as that used by engravers, but silvered 20 to prevent adherence of the copper deposit on the bare plate—and upon this surface we produce a picture in a medium somewhat resembling greasy ink, the ground representing the lights and the varying thicknesses of the 25 medium the various tones of the picture. From this work, after the treatment to be presently described, we make an electrotype plate from which impressions may be taken after the manner of copper-plate printing.

30 The mode of producing the picture may somewhat vary without affecting the ultimate result. One method which we have found efficient for certain kinds of artistic work, such as those which do not require much variation in tone, is to coat the ground-plate with the inking medium to a given depth or thickness by a printing-roller or equivalent means, and from this prepared surface to produce the picture by removing parts of the soft 35 coating where the lights and middle tints are required. This result may be effected by the aid of a piece of rag, a brush, or a piece of pointed wood, according to the character of the artistic touches desired. When the picture 40 is completed, a margin may be made by wiping the plate clean for a given distance inward from the edge thereof.

It will be understood that the work of the artist is to remove the coating to a less or 45 greater depth, as may be necessary to secure the requisite effects of light and shade, &c.

In place of first coating the plate and then

removing the inky compound to obtain the lights and middle tints, the reverse method may be employed, and with greater advantage 55 in respect of some classes of subjects where a breadth of light or medium tones prevail—that is to say, the artist will work upon the plate as if he were producing a tone-drawing, laying on the inky medium sparingly or otherwise to produce the varying tints and shadows required to give proper force and perspective to the picture. Thus the lights will be represented, as before, by the uncovered surface of the plate, the distances in the picture by 65 a sparse application of the medium employed, and the deepest tones by the greatest thickness of medium.

The picture produced in either of the above-mentioned ways, or it may be by the two 70 methods in combination, is next to be prepared for the electrotype-bath by giving it a metallic surface, on which the copper is to be deposited. In order, however, that the plate when obtained may hold the printer's ink in 75 its cavities, it is necessary to produce what is known as a "grain" in those parts of the plate, which grain must be coarser or finer, according to the depth of tint or tone required for the various parts of the composition. To produce this grain we dust over the picture while still tacky with a granulated or gritty material, which should be of various degrees of fineness. The granulated or gritty material which we have successfully used is a composition of powdered asphaltum and bronze powder in the proportion of two parts of the former and one of the latter. The composition, after careful mixing, is placed in a bag of fine muslin and then dusted over the picture 80 until the work of the artist is completely hidden. The surplus powder is then removed by a soft camel's-hair brush or its equivalent, and that which has come into contact with the picture is retained, the coarser grains being held by the thicker coating of the medium, while the films and thinner parts secure only 85 the finer grains. The picture in this state is laid aside for some three days to harden, and it is then ready for the bath. Care must, 90 however, be taken that the surface of the picture is not touched, as it is liable to injury from even a slight amount of pressure.

The electrotype is produced by electrodepo-

sition in the well-known manner, the picture having been by the dusting-over process converted into a properly-metallized surface.

The inky composition or medium which we employ for producing the picture consists of a vegetable oil—say boiled linseed-oil—mixed with German black or lampblack, with the addition of animal fat, which serves to retard the drying of the oil, the proportions being about equal parts, by weight, of oil, of German black or lampblack, and animal fat—say lard-oil.

The proportion of the animal fat will vary according to the nature of the picture in hand, it being essential that the thinner parts of the applied medium shall not harden during the progress of the picture.

The retention of the tackiness of the picture is especially necessary when a work of some elaboration is in hand, and some two, three or more days are required to complete it, the premature hardening of the medium preventing the proper attachment of the granulated mixture and thus rendering much of the artist's labor abortive. The electrotype of this plate will be an intaglio representing the reverse of the artist's work, and the impressions from the plate will therefore be a correct reproduction of the picture.

The plate may be used in the state in which it comes from the electrotype-bath to throw off impressions; but when the artist is familiar with the resources of the engraver the dry point may be used, or the processes of etching or mezzotint may be applied for working up the picture and producing brilliant artistic effects.

To increase the life of the plate it may be steel-surfaced in the manner commonly practiced with respect to engraved copper-plates.

It may be understood that in the composition with which the picture is dusted to produce the grain and prepare it for the electrotype-bath, the powdered asphaltum being inert to the action of the electrotype-bath only produces the grain and the bronze powder metallizes the surface to prepare it for the reception of the electrodeposit.

What we claim is—

1. The within-described method of producing artistic printing-surfaces in intaglio with a grain, consisting in first forming on a ground or base a picture having a greasy or tacky surface, next dusting over the surface of the picture while in a tacky state a granular substance possessing electrical conductivity and of different degrees of fineness, then removing the excess of the granular substance and finally subjecting the thus-coated picture to the electrotype-bath, as herein described.

2. The improvement in the method of producing printing-surfaces in intaglio with a grain, consisting in first forming on a ground or base a picture in a greasy or tacky medium, next dusting over the surface of the picture a granular composition consisting of a powder of different degrees of fineness inert to the electrotype-bath and a metallic powder, then removing the excess of the granular composition, and finally subjecting the thus-coated picture to the electrotype-bath, as herein described.

London, March 14, 1895.

HUBERT HERKOMER.  
HENRY THOMAS COX.

Witnesses:

H. K. WHITE,  
W. M. HARRIS.